# EUROPEAN PATENT SPECIFICATION

(11) **EP 0 010 764 B1**
(45) Date of publication and mention of the grant of the patent: **01.02.1984**
(21) Application number: 79104267.4
(22) Date of filing: 02.11.1979
(51) Int. Cl.: D06M 13/16, C10M 1/08, D06M 13/18, D06M 13/26, D06M 13/34

(54) **Polypropylene yarn product of improved stability and method for preparing a textile material**
Polypropylengarnerzeugnis mit verbesserter Stabilität sowie Verfahren zur Herstellung eines Textilmaterials
Produit filé en polypropylène ayant une stabilité améliorée et méthode de traitement d'un matériau textile

(30) Priority: 06.11.1978 US 957786
(43) Date of publication of application: 14.05.1980
(73) Proprietor: PHILLIPS PETROLEUM COMPANY, Bartlesville Oklahoma 74004 (US)
(72) Inventor: Taylor, Peter Anthony, Greenville, South Carolina (US)
(74) Representative: Dost, Wolfgang, Dr.rer.nat., Dipl.-Chem.

## Description

In the formation of textile materials from melt spun polypropylene it is normally necessary to apply a finishing composition to the filaments, yarns and other textile embodiments thereof to make such materials more amenable to the various operations to which they are subjected during processing, for example, spinning, winding, yarn-forming, weaving or knitting, and to improve the properties of the finish products. In the processing of the textile materials, the finishing composition is intended to reduce friction between the yarn and various pieces of equipment with which it comes into contact, such as guides, rollers and the like, and in both the processing and use of the textile materials to reduce friction between the fibers themselves, to prevent fiber and yarn breakage and to minimize excessive attraction or repulsion of the filaments caused by electrostatic charges. Accordingly, such finishing compositions usually contain a lubricant and an antistatic agent. Various other additives such as bactericides or corrosion inhibitors, may also be added to the finishing composition.

However, it has been found that not all thermoplastic materials respond to finishing compositions in the same manner, not all combinations of finishing agents are compatible with one another and not all finishing agents are compatible with stabilizers added to the thermoplastic melt.

For example, ethoxylated lubricants have heretofore been found to be highly superior to conventional textile lubricants when utilized in finish compositions for treating melt spun polypropylenes. Accordingly, it is highly desirable to utilize these synthetic lubricants in the finish composition. However, it has been found, in accordance with the present invention, that polypropylenes do not respond to ethoxylated lubricants in the same manner as other thermoplastic fiber-forming materials, when they contain a stabilizer system comprising a hindered phenol in an amount of from 0.1 to 0.6 weight percent total stabilizers, i.e. less than the normal amounts of stabilizers. Rather, it has been found that some antagonistic reaction occurs between an ethoxylated lubricant and the hindered phenol which results in decreasing the thermal, light and/or color stability of the polypropylene textile products.

Accordingly, the invention relates to a polypropylene yarn product of a melt spun polypropylene formed from a melt containing from 0.1 to 0.6 weight percent total stabilizer including a hindered phenol, and having applied thereto a finish composition comprising an ethoxylated textile lubricant and an antistatic agent, which is characterized in that said antistatic agent is a phosphate ester. Furthermore, the invention relates to a process for preparing a polypropylene textile material comprising (a) melt spinning polypropylene filaments from a melt containing from 0.1 to 0.6 weight percent total stabilizer including a hindered phenol and (b) applying to said melt spun polypropylene a finish composition comprising an ethoxylated textile lubricant and a phosphate ester.

The yarn may also be draw-twisted before or after the packaging of the yarn. Such draw-twisted yarns may be woven into products particularly suitable for use as dye bags, laundry bags, and the like.

It has been found, in accordance with the present invention, that, by including significant amounts of at least one phosphate ester in a textile finish composition containing an ethoxylated lubricant, the stability of polypropylene textile materials can be substantially improved. It has also been found that, in many cases, the color stability of such polypropylene textile materials can also be improved by the specified combination of ethoxylated lubricant and antistatic agent. The finish composition optionally, but desirably, contains minor amounts of a bactericide and may also contain minor amounts of other additives such as corrosion inhibitors and the like.

While the finish composition may be applied to the textile materials at any time during the processing thereof, it is preferably applied to the filaments as soon as they have set, so that the full benefit of the stabilizing properties thereof can be realized during the later processing thereof. Thus, in accordance with this embodiment, there are produced as-spun polypropylene yarns of highly improved thermal stability and in many cases of improved light and/or color stability.

In a preferred embodiment of the present invention, the yarns thus produced are draw-twisted and again packaged. The draw-twisting can also be applied in a continuous process prior to the initial winding or packaging of the yarn. The draw-twisted yarns have been found to be highly effective for the production of dye bags, laundry bags and the like when woven and formed into appropriate articles.

The polypropylene textile materials to which the present invention is directed are homopolymers of propylene and copolymers of propylene and another aliphatic 1-olefin containing 2 to 8 carbon atoms, in which the comonomer constitutes up to about 20 mole percent of the copolymer.

The ethoxylated textile lubricants utilized in accordance with the present invention include any of the known ethoxylated lubricants such as polyethylene glycols, mixed polyethylene-propylene glycols, monoalkyl esters of mixed polyethylene-polypropylene glycols, ethoxylated esters of fatty acids, rosin acids and tall oil acids, ethoxylated castor oils or ethoxylated hydrogenated castor oils. More specific examples are ethoxylated aliphatic alcohols, ethoxylated alkylphenols, ethoxylated sorbitan (anhydro- sorbitol) esters, ethoxylated sorbitol esters, ethoxylated glycerol esters, ethoxylated pentaerythritol esters, ethoxylated fatty acids, ethoxylated fatty acid amides, ethoxylated-propoxylated fatty acids, ethoxylated-propoxylated fatty acid esters, ethoxylated-propoxylated castor oils, ethoxylated-propoxylated hydrogenated castor oils, ethoxylated-propoxylated aliphatic alcohols and ethoxylated-propoxylated alkyl phenols.

Presently preferred ethoxylated lubricants include the random copolymers of the monobutyl ether of poly(oxyethylene-oxy-1,2-propylene) having viscosities in terms of Saybolt Universal Seconds (SUS) at 100°F (38°C) ranging from 170 to 5100 and even more preferably from 250 to 3500, the methyl ether of poly(oxyethylene-oxy-1,2-propylene) laurate wherein the number of moles of combined ethylene oxide, is about 7 and the number of moles of combined propylene oxide is about 2, and the isododecyl ether/poly(oxyethylene) adduct wherein the number of moles of combined ethylene oxide is about 6 per mole hydrophobe.

A more complete description of the ethoxylated lubricants is given in Kirk-Othmer, Encyclopedia of Chemical Technology, 2nd Edition 19, 531-554 (1969). A more complete description of the polyethylene glycols, etc. is given in volume 10, pages 654-659 of the reference encyclopedia.

The hindered phenols are utilized as thermal stabilizers or antioxidants. Such materials are known in the art.

Typical of such stabilizers are 2,6-di-t-butyl-4-methylphenol (BHT); octadecyl [3-(3,5-di-t-butyl-4-hydroxyphenyl)] propionate (irganox (TM) 1076, Ciba-Geigy Chemical Co.); tetrakis[methylene(3,5-di-t-butyl-4-hydroxyhydrocinnamate)] methane (Irganox (TM) 1010, Ciba-Geigy Chemical Co.), di-n-octadecyl(3,5-di-t-butyl-4-hydroxybenzyl)phosphonate; 1,3,5-trimethyl-2,4,6-tris(3,5-di-t-butyl-4-hydroxybenzyl) benzene and tris(3,5-di-t-butyihydroxybenzy))isocyanurate.

The phosphate ester antistatic agent utilized in accordance with the present invention includes hydrocarbyl phosphate esters, ethoxylated hydrocarbyl phosphate esters, partially hydrolyzed hydrocarbyl phosphate esters or their salts. By hydrocarbyl is meant a hydrocarbon radical selected from the alkyl, cycloalkyl, aryl and combinations thereof such as alkyllauryl, containing from 1 to 20 C atoms. Usually a mixture of di- and monoalkyl esters is utilized but the composition is also effective when completely esterified phosphoric acid compounds are employed. It has also been found that the use of these phosphate esters is quite effective in inhibiting color formation during gas fired heat treatments. It has further been found that the inhibition of color formation is influenced by the pH and the neutralizing cations employed. The lower the pH the less colour produced. Preferably, the pH is maintained between 3 and 9 and preferably between 4 and 7. The preferred phosphate esters are the partially neutralized acid esters of phosphoric acid or the equivalent partially hydrolyzed triesters of phosphoric acid. The present order of neutralizing cations has been found to be ammonium, mono-, di-and triethanolammonium, lithium, sodium and potassium. The potassium was found to be the least desirable, although useable in accordance with the present invention.

The finish composition of the present invention also desirably contains a bactericide such as 6-acetoxy-2,4-dimethyl-m-dioxane (Givgard DXN@, Givuadan Corp., Clifton, NJ).

In the finish composition of the invention the ethoxylated lubricant is utilized in amounts between 50 and 98 percent by weight of the finish composition, preferably between 60 and 95 percent by weight of the composition. The balance of the finish composition is preferably the antistatic agent which is used in amounts between 2 and 50 percent by weight, preferably between 5 and 40 percent by weight of the finish composition. The bactericide may be present in amounts up to about 1.0 percent by weight of the final composition and like minor amounts of other suitable additives may be included, such as corrosion inhibitors.

A preferred embodiment of the present invention will be illustrated by reference to the accompanying drawings.

In accordance with Figure 1, the polypropylene melt is extruded from a plural orifice spinneret 2, of conventional design. While spinneret 2 is shown in the drawings as producing a single threadline it is obvious that the spinneret may produce two or more threadlines. The filaments from spinneret 2 are passed through a conventional quench zone 4 where the filaments are cooled and set. Finish is applied by conventional finish applicator means 6 which may take any appropriate form. For example, a "kiss" roll may be utilized to apply finish to the filaments as a gathered threadline or yarn or as a band spread across the finish roll. A slot type finish applicator could also be utilized, the only requirement being that the finish be uniformly applied to the filaments or yarn. The yarn is then wound on an appropriate conventional winder 8 to form a yarn package 10. Appropriate guides, guide rolls, godet rolls, and the like will of course be utilized. The process as illustrated in Figure 1 produces a yarn in its as-spun state. However, it is also possible to draw-twist the yarn before winding the same on package 10. Whether draw-twisting is practiced as a part of the spinning operation will depend to some extent upon whether the yarn is partially oriented yarn or a conventional undrawn yarn. Normally it is considered that winder takeup speeds in excess of about 1500 meters per minute will produce a partially oriented yarn whereas takeup speeds of less than about 1500 meters per minute, for example about 800 meters per minute, produce an unoriented or undrawn yarn.

Figure 2 illustrates a preferred draw-twisting operation in accordance with the present invention. In Figure 2 yarn is withdrawn from yarn package 10 by means of the draw means 12 made up of conventional draw rolls, 12a and 12b, respectively. Thereafter, twist means 14 conventionally applies by means of a flyer 16 as it is wound on package 18. Obviously any appropriate drawing and twisting apparatus may be utilized. It will also be apparent to one skilled in the art that the system would include appropriate guides, guide rolls, draw heaters, etc.

The draw-twisted yarn when converted into an appropriate fabric and formed into a bag or the like has been found to make excellent dye bags, laundry bags and the like. The resultant products have superior temperature stability compared with conventionally finished textile materials of polypropylene and to conventional dye bag textiles. In addition, certain of the polypropylenes have been found to have superior inhibition to color formation as compared with conventionally finished polypropylenes and commercially available dye bag textiles.

The following examples will illustrate the advantages of the present invention.

### Example 1

The stability of polypropylene yarns with and without the phosphate-type antistatic agents was determined in laundering cycle tests in the present example.

In this test, a polypropylene melt composition was prepared by adding to the polypropylene 0.05 parts by weight per 100 parts of polypropylene (phr) of calcium stearate, 0.3 phr tris(3,5-di-t-butyl- hydroxybenzyl)isocyanurate, 0.1 phr hydrolysis resistant distearyl pentaerythritol disphosphite, 0.1 phr trilauryl trithiophosphite and about 0.375% titanium oxide. The polypropylene had a melt flow of 12 and when combined with the specified stabilizing system is designated hereinafter as resin B.

The finish designated in Table 1 below as finish I contains the following:
90 wt. % ethoxylated coconut acid (9 moles ethylene oxide per mole acid).
10 wt. % ethoxylated coconut amino ethanolamine (3 moles ethylene oxide per mole coconut derivative) - commercially available ethoxylated lubricants.

The finished designated as finish II contains the following:
Lubricant
32.15% methyl ether of poly(oxyethylene-[7-moles]oxy-1,2-propylene[2 moles]) laurate (Imperial Chemical, Inc., TL 1038).
32.15% poly(oxyethylene[6.5 moles]), isodecyl alcohol ether (Imperial Chemical, Inc. TL 1074).
19.4% butyl ether of random copolymer, poly(oxyethylene-oxy-1,2-propylene) having SUS viscosity of 2000 (Union Carbide Co.).

Antistatic agent
13.19% mixture of di- and mono-hexyl phosphoric acid (Imperial Chemical, Inc. G2199). 2.05% NaOH.
0.96% diethanolamine.

Bactericide
0.1 % 6-acetoxy-2,4-dimethyl-m-dioxane (Givgard DXN, Givaudan Corp. Clifton, N.J.).

The specified finishes were applied to the yarns at a rate of 3.6 to 4.5 weight % solids based on the weight of yarn.

In the test, the yarn was knitted into a sleeve and the sleeve trimmed so that the yarn could be easily unravelled for sampling. The sleeve, weighing about 5 grams, was placed in a 500 milliliter, flat bottom flask fitted with a water cooled reflux condenser. 200 milliliters of a 0.2% AATCC Standard Soap Solution was boiled under reflux for 6 hours after which time the sleeve was removed, rinsed free from the solution and squeezed dry. The sleeve was then dried for 15 hours at 130°C in an electrically heated, forced air oven to complete the cycle. About a 5 foot (1.5 m) sample of the yarn was removed from the sleeve and tested for strength and elongation retention on an Instron Tensile Tester after 3, 5 and 8 cycles, respectively.

The results of this test are set forth in Table 1 below:

UV-stability

The ultraviolet stability of the polypropylene yarns referred to in Table 1 above was also tested.

The ultraviolet stability was measured by exposing 2" by 3" (5.1 by 7.6 cm) knitted sleeves mounted on black backed Atlas mounting fadeometer cards. Degradation is either when the fabric tears or when the fabric flakes while being gently scratched with a fingernail. Usually if the sleeve is of fine denier yarn the fabric will tear and it is the sleeve surface closest to the black backing which tears before the surface closest to the arc. With heavier denier fabrics flaking of the surface facing the arc usually occurs before the fabric can be torn. Table 2 below gives the results of these tests.

It is obvious from the above examples that finishes containing an ethoxylated lubricant and the phosphate-type antistatic agents, in accordance with the present invention, (finish II) were vastly superior to finishes containing only ethoxylated lubricants and balanced finishes containing the ethoxylated lubricants and antistatic agents other than the phosphate-type antistatic agents utilized in accordance with the present invention, which other lubricant compositions have been highly successful as finishes for other textile materials.

### Example 2

In this example the finish compositions of the present invention were tested for use as dye bag yarns. The yarns were made from a stabilized polypropylene melt designated resin B in Example 1 and were finished with either finishes I or II as specified in the previous examples. The finish was metered onto the yarn with no problems. The yarn was draw-twisted using a standard 1680/280 yarn process. Eight positions of a draw twister processing 1680/280 yarns were used. Again no problems were seen. The yarns were then coned into ten ounce (280 g) packages and knitted into dye bags for testing.

The following tests were made:
Stability to up to 8 cycles of an accelerated mock dyeing test.
Stability up to 8 cycles of an accelerated laundering test.
Stability to C-Arc fadeometer exposure test.
Stability to GMB-Arc fadeometer exposure test.
Accelerated gas fade color development test.
AATCC gas fade color development test.

In addition to testing yarn with finish II of the present invention and the yarn with finish I as a control, in some cases competitive dye bag yarns, designated C, were tested for comparison.

The mock dye cycle test is the same as the previously described laundering cycle except that the treating solution was 200 milliliters of the following:
0.3% Alkanol ITM) ND (Dupont) - sodium alkyl diaryl sulfonate.
0.16% Merpol^{(TM)} OJS (Dupont) - ethylene oxide condensate.
0.3% MSP - monosodium phosphate.

The GMC-Arc fadeometer exposure test was substantially the same as the previously described carbon arc fadeometer test.

The accelerated gas fade color development test simulates processes which involve heating and curing or drying in gas fired ovens. It also produces colors which have been seen transiently under the same kinds of storage conditions which have not heretofore been simulated. The test provides for a 10 minute heating cycle at 130°C followed by a 2-hour treatment in an atmospheric fume chamber (AATCC test method 23-1975).

The regular gas fade test is described in AATCC test method 23-1975.

The results were recorded and the percent toughness retained was calculated for each sample. The toughness is defined as:

The results of this series of tests are set forth in Tables 3, 4, 5 and 6 below:

The above results are analyzed below.

Selection of commercial dye bag yarn C having a 165/35 denier for the quantitative strength retention test was made on the basis of laundering cycle tests in which three commercial dye bag yarns from the same manufacturer were cycled to failure. The commercial yarn having a denier of 165/35 was found to be the most stable of the three yarns tested (see Table 5 above).

In the quantitative dyeing/laundering simulations it is the elongation which is most rapidly affected, the toughness factor is used as the critical criterion because it balances the elongation and the tenacity into a property which has been found to be the equivalent to performance in actual practice.

Although the color of the yarns has not been quantitatively evaluated, the dye bag yarns in accordance with the present invention are whiter than the control yarn and than the commercial dye bag yarn; it remains whiter in the cycling test, the thermal stability tests and in actual laboratory storage experiments. Accelerated gas fade tests showed no pinking problems with the dye bag yarns of the present invention and no such problems have been observed with the control yarns. In 3-cycle gas fade tests, the yarns show quite a severe color development. However, this is not believed to be a problem in dye bag yarns since the only place it will slow up is after long storage in a high nitrogen oxide atmosphere. The dye bag yarns would not be subjected to such an environment since legislation has essentially ruled out this kind of contamination.

### Example 3

Tests were also conducted utilizing a 12 melt flow polypropylene melt composition stabilized with 0.30% distearylthiodipropionate, 0.10% tetrakis[methylene(3,5-di-t-butyl-4-hydroxy hydrocinnimate)] methane and 0.05% calcium stearate and a 12 melt flow polypropylene having a stabilizer system; comprising, 0.30% distearylthiodipropionate, 0.10% tetrakis[methylene13,5-di-t-butyl-4-hydroxy hydrocinnimate)] methane (Irganox(TMI 1010, Ciba-Geigy), 0.05% calcium stearate and 0.10% hydrolysis resistant distearyl pentaerythritol diphosphate Weston^{(TM)} 619, a product of Borg-Warner Chemicals, Parkersburg, W. Va. Both of the stabilizing systems utilized in the polypropylene melt composition are seen to contain hindered phenols. It was found that about 2% of an ethoxylated textile lubricant applied to these textile materials will reduce the thermal stability at 130°C from 400 hours to 60 hours or from 1500 hours to 200 hours depending on the denier of the product. However, the presence of about 10% to 50% of the phosphates of the present invention and the same ethoxylated lubricants the textile materials recover substantially all of the strength thus lost.

It was also found that a further benefit from the use of the finish compositions of the present invention is attained when the polypropylene melt composition contains a hindered phenol. Specifically, inhibition of color formation during gas fired heat treatments is improved. For example, yarns spun from resin formulations B and C above when heated to 130°C and exposed for 2 hours in a nitrogen oxide gas fade oven will turn pink. This pink color will be increased in the presence of an ethoxylated textile lubricant-containing finish unless the finish has added thereto a phosphate type antistatic agent as taught in the present invention.

## Claims

1. A polypropylene yarn product of a melt spun polypropylene formed from a melt containing from 0.1 to 0.6 weight percent total stabilizer including a hindered phenol, and having applied thereto a finish composition comprising an ethoxylated textile lubricant and an antistatic agent, characterized in that said antistatic agent is a phosphate ester, said ethoxylated textile lubricant (a) and said phosphate ester (b) being contained in amounts of 50-98 percent by weight of (a) and 2-50 percent by weight of (b), each based on the finish composition.

2. The product of claim 1 characterized in that the finish composition additionally contains a bactericide.

3. The product of claim 1 characterized in that the phosphate ester is an at least partially neutralized acid ester of a phosphoric acid.

4. The product of claim 3 characterized in that said partially neutralized acid phosphate ester exhibits a pH between 3 and 9.

5. The product of claim 3 characterized in that the acid phosphate ester is neutralized with a neutralized composition including ammonia.

6. The product of claim 3 characterized in that the acid phosphate ester is neutralized with a material selected from monoethanolamine, diethanolamine, triethanolamine, sodium hydroxide, lithium hydroxide, ammonium hydroxide and mixtures thereof.

7. The product of claim 1 characterized in that the phosphate ester is an ethoxylated alkyl phosphate ester.

8. The product of any of claims 1 to 7 characterized in that the yarn product is a draw-twisted, melt spun polypropylene.

9. The product of claim 1 characterized in that said ethoxylated textile lubricant (a) and said phosphate ester (b) are contained in amounts of 60-95 percent by weight of (a) and 5-40 percent by weight of (b), each based on the finish composition.

10. A process for preparing a polypropylene textile material comprising:
a) melt spinning polypropylene filaments from a melt containing from 0.1 to 0.6 weight percent total stabilizer including a hindered phenol, and
b) applying to said melt spun polypropylene a finish composition as defined in one of claims 1 to 8.

11. The process of claim 10 characterized in that the melt spun polypropylene is formed into a yarn and the yarn is draw-twisted.

12. The process of claim 11 characterized in that the finish composition is applied to the melt spun filaments shortly after they have set.

## Revendications

1. Produit en filé de polypropylène constitué d'un polypropylène filé à l'état de masse fondue, formé à partir d'une masse fondue contenant 0,1 à 0,6% en poids de stabilisant total comprenant un phénol à empêchement stérique, et auquel on a appliqué une composition de produits de finissage contenant un lubrifiant éthoxylé pour textile et unagent antistatique, caractérisé en ce que l'agent antistatique est un ester formé de phosphate, le lubrifiant éthoxylé pour textile (a) et l'ester formé de phosphate (b) étant contenus en quantité de 50-98% en poids de (a) et 2-50% en poids de (b), chacun basé sur la composition de produit de finissage.

2. Produit selon la revendication 1, caractérisé en ce que la composition de produit de finissage contient en outre un bactéricide.

3. Produit selon la revendication 1, caractérisé en ce que l'ester formé de phosphate est un ester d'acide au moins partiellement neutralisé, d'un acide phosphorique.

4. Produit selon la revendication 3, caractérisé en ce que l'ester formé de phosphate d'acide partiellement neutralisé présente un pH entre 3 et 9.

5. Produit selon la revendication 3, caractérisé en ce que l'ester formé de phosphate d'acide est neutralisé avec une composition de neutralisation comprenant de l'ammoniac.

6. Produit selon la revendication 3, caractérisé en ce que l'ester formé de phosphate d'acide est neutralisé avec une matière choisie parmi la monoéthanolamine, la diéthanolamine, la triéthanolamine, la soude, la lithine, l'ammoniaque et leurs mélanges.

7. Produit selon la revendication 1, caractérisé en ce que l'ester formé de phosphate est un ester formé de phosphate d'alkyle éthoxylé.

8. Produit selon l'une quelconque des revendications 1 à 7, caractérisé en ce que le produit formé de filé est un polypropylène filé à l'état de masse fondue, soumis à une fausse torsion.

9. Produit selon la revendication 1, caractérisé en ce que le lubrifiant éthoxylé (a) pour textile et l'ester formé de phosphate (b) sont contenus en quantités de 60-95% en poids de (a) et 5-40% en poids de (b), chacune basée sur la composition de produit de finissage.

10. Procédé de préparation d'une matière textile en polypropylène consistant:
a) à filer à l'état de masse fondue des filaments de polypropylène à partir d'une masse fondue contenant 0,1 à 0,6% en poids de stabilisant total comprenant un phénol à empêchement stérique, et
b) à appliquer au polypropylène filé à l'état de masse fondue une composition de produit de finissage selon l'une quelconque des revendications 1 à 8.

11. Procédé selon la revendication 10, caractérisé en ce que le polypropylène filé à l'état de masse fondue est transformé en un filé et le filé est soumis à une fausse torsion.

12. Procédé selon la revendication 11, caractérisé en ce que la composition de produit de finissage est appliquée aux filaments filés à l'état de masse fondue peu de temps après qu'ils ont été stabilisés.

## Patentansprüche

1. Polypropylen-Garnerzeugnis aus schmelzgesponnenem Polypropylen, gebildet aus einer Schmelze, die 0,1 bis 0,6 Gewichtsprozent Gesamtstabilisator einschließlich eines sterisch gehinderten Phenols enthält, und mit einem aufgebrachten Finish, das ein ethoxyliertes Textil-Gleitmittel und ein antistatisches Mittel enthält, dadurch gekennzeichnet, daß das antistatische Mittel ein Phosphorsäureester ist und das ethoxylierte Textil-Gleitmittel (a) und der Phosphorsäureester (b) in Mengen von 50 bis 98 Gewichtsprozent (a) und 2 bis 50 Gewichtsprozent (b), jeweils bezogen auf das Finish anwesend sind.

2. Erzeugnis nach Anspruch 1, dadurch gekennzeichnet, daß das Finish zusätzlich ein Bakterizid enthält.

3. Erzeugnis nach Anspruch 1, dadurch gekennzeichnet, daß der Phosphorsäureester ein zumindest teilweise neutralisierter saurer Ester einer Phosphorsäure ist.

4. Erzeugnis nach Anspruch 3, dadurch gekennzeichnet, daß der teilweise neutralisierte saure Phosphorsäureester einen pH-Wert von 3 bis 9 besitzt.

5. Erzeugnis nach Anspruch 3, dadurch gekennzeichnet, daß der sauer Phosphorsäureester mit einem Neutralisationsmittel, das Ammoniak einschließt, neutralisiert ist.

6. Erzeugnis nach Anspruch 3, dadurch gekennzeichnet, daß der saure Phosphorsäureester mit Monoäthanolamin, Diäthanolamin, Triäthanolamin, Natriumhydroxid, Lithiumhydroxid, Ammoniumhydroxid, oder Gemischen hiervon, neutralisiert ist.

7. Erzeugnis nach Anspruch 1, dadurch gekennzeichnet, daß der Phosphorsäureester ein ethoxyliertes Alkylphosphat ist.

8. Erzeugnis nach einem der Ansprüche 1 bis 7, dadurch gekennzeichnet, daß das Garnerzeugnis ein streckgezwirntes, schmelzgesponnenes Polypropylen ist.

9. Erzeugnis nach Anspruch 1, dadurch gekennzeichnet, daß das ethoxylierte Textil-Gleitmittel (a) und der Phosphorsäureester (b) in Mengen von 60 bis 95 Gewichtsprozent (a) und 5 bis 40 Gewichtsprozent (b), jeweils bezogen auf das Finish, anwesend sind.

10. Verfahren zur Herstellung eines Polypropylen-Textilierzeugnisses durch
a) Schmelzspinnen von Polypropylen-Filamenten aus einer Schmelze, die 0,1 bis 0,6 Gewichtsprozent Gesamtstabilisator, einschließlich eines sterisch gehinderten Phenols enthält, und
b) Aufbringen eines Finish nach einem der Ansprüche 1 bis 8 auf das schmelzgesponnene Polypropylen.

11. Verfahren nach Anspruch 10, dadurch gekennzeichnet, daß das schmelzgesponnene Polypropylen zu einem Garn verarbeitet und das Garn einer Streckzwirnung unterworfen wird.

12. Verfahren nach Anspruch 11, dadurch gekennzeichnet, daß das Finish auf die schmelzgesponnenen Filamente kurz nach deren Verfestigung aufgebracht wird.
